

## UNITED STATES PATENT OFFICE

2,180,971

## WATERPROOFING COMPOSITION

Arthur F. Taggart, Scarsdale, and Warley L. Parrott, New York, N. Y.

No Drawing. Application April 22, 1937,  
Serial No. 138,364

4 Claims. (Cl. 134—13)

Our invention relates to waterproofing compositions, and more particularly to waterproofing compositions that form, upon evaporation of their volatile constituents, fine-grained to glass-like 5 water-repellent films.

One of the features of our invention is the crystallization of a water-repellent crystalline material in the composition controlled by a non-crystalline water-repellent constituent present in thickened form, whereby the normal growth of the crystals of the controlled material is arrested and that material deposits in the form of extremely fine size crystals. These fine crystals uniformly and intimately admix with the fine size particles of the controlling non-crystalline substance to form upon complete solidification a continuous fine-grained to glass-like film the imperforate nature of which prevents moisture penetration.

Preliminarily to the discovery upon which our invention is based, we prepared and observed microscopically numerous slides of different mixtures of water-repellent substances and tested these mixtures for comparative waterproofing effectiveness. We observed from these tests that the most effective waterproofing mixtures, whatever the ingredients used, were those that produced uniform fine-grained to glass-like films. Such films, generally speaking, are composed of ingredients that are so finely divided that no definite crystalline structure can be detected in the film when it is viewed through a microscope with dark field illumination and having a magnification of about 150 diameters.

Following these observations, we discovered that highly efficient waterproofing compositions capable of producing the desired fine-grained to glass-like films may be consistently produced by admixing in the proper proportions an organic solvent, an organic water-repellent crystal-forming material, and a water-repellent substance that will cause the solvent and this substance to thicken sufficiently, before the crystallizable material begins to crystallize, to arrest the growth of crystals when the crystallizable material begins to solidify upon continued evaporation of the solvent. More specifically, we found that in order to effect the desired crystal growth control the concentration of the crystallizable material must be less than that at which the solvent would be super-saturated with that material before the thickener and solvent has thickened.

An object of our invention is to provide a

waterproofing composition containing an intimate admixture of various water-repellent constituents so related in solubility in the solvent used and in concentration therein, that whatever the constituents used the composition will form, upon evaporation of its volatile constituents, a highly water-repellent fine-grained to glass-like film.

From the numerous microscopic observations that we have made of various waterproofing compositions, we have noticed that if the composition does not contain, at the time of crystallization of the crystallizable water-repellent constituents, a constituent that will interfere with the normal crystal growth of the crystallizable material, the latter will deposit in the form of relatively large, irregular and separated crystals. The films produced by such compositions are non-uniform and have a porphyritic or perforated structure that permits moisture penetration. These films are not satisfactory since they do not completely waterproof the materials to which they are applied. On the other hand, we have found that if the solvent and water-repellent constituents are properly chosen and their concentrations properly regulated to effect the above mentioned crystal growth interference, the compositions will produce upon solidification uniform, fine-grained to glass-like, imperforate, highly water-repellent films.

The rule or formula to be followed for producing the improved waterproofing compositions of our invention comprises selecting an organic solvent, a crystallizable water-repellent material, and a normally solid or viscous substance (preferably water-repellent) and that is chemically or physically so related that the mixture of this substance and the solvent will thicken upon concentration thereof; and to so proportion them that the thickening will occur before the crystallizable water-repellent constituent or constituents in the liquid waterproofing composition begin to crystallize. In other words, when the waterproofing composition is applied to a material to be waterproofed and the organic solvent begins to evaporate, one of the constituents must first cause this substance and the solvent to thicken, either in the form of a gel or a viscous mass, so that when the crystallizable water-repellent material subsequently begins to precipitate out of solution the thickener and solvent will be in thickened form to arrest the normal crystal growth of the precipitate so that the crystals of water-repellent material will be deposited in extremely fine size form, con-

ducive to uniform intimate admixture with the normally fine size or amorphous particles of the water-repellent thickener to produce upon the material to be waterproofed a composite fine-grained to glass-like water-repellent film.

One of the important and commercially valuable features of our invention is that the waterproofing composition may be made from any two or more water-repellent constituents and a suitable solvent properly selected from large groups of such constituents subsequently denoted herein and, in general, the same degree of waterproofing effectiveness will be obtained in each case. Regardless of the constituents so selected, their maximum waterproofing effectiveness will always be produced so long as the crystallization of the crystallizable water-repellent material is properly controlled to produce very fine size crystals and thereby fine-grained films. Accordingly, a number of water-repellent constituents which heretofore have been considered in some respects undesirable, such as for example, paraffin, waxes, and gums, may now be used as constituents in highly effective waterproofing compositions. As a result, the field of effective waterproofing compositions has been markedly extended.

While the exact water resistance of compositions produced from various mixtures of the selected water-repellent constituents will vary somewhat inherently, they will each possess a high degree of water-repellency because of the fine-grained, uniform, compact structure of their deposited films. That is to say, these films are composed of extremely small particles so uniform in size, admixture and distribution that the film is practically homogeneous and substantially free of interstices. Consequently, the film offers a uniform high resistance to water over its entire surface and being practically non-porous it is impervious to water penetration.

In view of the fact that the only essential requirement for producing the desired type of waterproofing composition is proper selection of a water-repellent substance that with the solvent will thicken sufficiently at the proper concentrations to arrest the crystal growth of the water-repellent crystallizable material, it will be apparent that wide variations may be made in the several constituents used in the waterproofing composition as illustrated by the following.

The crystallizable water-repellent material, which constitutes one of the principal waterproofing ingredients in the composition, may be any organic water-repellent material that will crystallize upon concentration in an organic solvent. Some of the water-repellent crystallizable materials that we have found satisfactory are as follows:

60 Fatty materials, e. g., both those natural fats and the artificially saturated animal, vegetable and marine fats and oils which crystallize and are substantially solid at normal atmospheric temperatures; such as lard, tallow, cocoa butter, fish 65 and whale fats, hydrogenated animal oil, cotton seed, corn, cocoanut, peanut, fish and whale oils.

Fatty acid glycerides, e. g., both those natural glycerides and those artificially saturated glycerides of the higher fatty acids found in animal, vegetable and marine fats which crystallize and are substantially solid at normal atmospheric temperatures, e. g., hydrogenated fish oil glycerides.

Higher fatty acids; e. g., both those natural acids and those artificially saturated fatty acids

found in animal, vegetable and marine fats, which crystallize and are substantially solid at normal atmospheric temperatures, e. g., stearic acid, hydrogenated fish oil acids.

Natural and artificial waxes; e. g., carnauba, 5 wool wax, bee's wax.

Higher alcohols and ketones, e. g., cetyl, ceryl, melissyl alcohols, and others which are substantially solid at normal atmospheric temperatures, e. g., cholesterol, and camphor.

Hydrocarbons; e. g., paraffin, montan, ceresin, and others which are substantially solid at normal atmospheric temperatures.

The solvent used may be any one of the organic evaporative solvents that will act as a common solvent for the water-repellent thickener and the crystallizable material; and with the thickener will thicken upon evaporation of the solvent before the concentration of the crystallizable material in the mixture becomes high enough for 20 the precipitation of the crystallizable material to start. Examples of solvents that we have found satisfactory are as follows:

1. Petroleum distillates of relatively high saturation in the gasoline-kerosene boiling range; 25 e. g., petroleum naphtha, paraffin oil (kerosene)

2. Light aromatic hydrocarbons and substituted derivatives; e. g.,

|              |    |
|--------------|----|
| Benzol       | 30 |
| Tolulol      |    |
| Xylool       |    |
| Nitrobenzene |    |

3. Oils derived by steam distillation of resinous woods; e. g., turpentine

4. Halogen derivatives of lower hydrocarbons; 35 e. g.,

|                      |    |
|----------------------|----|
| Carbon tetrachloride | 40 |
| Chloroform           |    |
| Ethylene-dichloride  |    |

#### 5. "Cellosolve"

The thickener may be any organic, preferably waterproof, substance that with the solvent will thicken at the proper concentration to arrest the crystal growth of the crystallizable water-repellent material. We have found it advantageous to use water-repellent substances as thickeners. These substances are of the type normally considered as amorphous, although X-ray analyses might show some or all of these substances to have, at least in part, a crystalline structure. We appreciate that any waterproof substance whether of an organic or inorganic nature and whether of a crystalline or non-crystalline character, could be used as the thickener in accordance with our invention provided it served the purpose of controlling the crystal growth of the definitely crystalline water-repellent material or materials used in the composition. The principal requirement for the thickener is that regardless of its chemical nature, the solvent and the thickener it will increase in viscosity at the proper concentration and time to effect the desired crystal growth control. The thickener may be either of a gel-forming type or of a non-gel-forming type. As far as the physical character of the thickener is concerned, it is only necessary that it and the solvent will be sufficiently viscous to physically interfere with the normal crystal growth of the crystallizable water-repellent material.

Examples of thickeners that we have found satisfactory for use in our invention are the following:

*Example VI*

|                                                                                                        |       |       |
|--------------------------------------------------------------------------------------------------------|-------|-------|
| Collodion solution consisting of tetra-nitrate of cellulose, ethyl alcohol and ethyl ether (thickener) | c. c. | 5     |
| Cholesterol (crystallizable material)                                                                  | gram  | 0.025 |

*Example VII*

|                                                                                                        |       |     |
|--------------------------------------------------------------------------------------------------------|-------|-----|
| Collodion solution consisting of tetra-nitrate of cellulose, ethyl alcohol and ethyl ether (thickener) | c. c. | 10  |
| Camphor (crystallizable material)                                                                      | gram  | 0.3 |

*Example VIII*

|                                                            | Per cent |    |
|------------------------------------------------------------|----------|----|
| Aluminum stearate (thickener)                              | 3        | 15 |
| Cumar (thickener)                                          | 5.0      |    |
| Hydrogenated fish oil glycerides (crystallizable material) | 2.7      |    |
| Hydrogenated fish oil acids (crystallizable material)      | 0.3      | 20 |
| Hydrogenated naphtha (solvent)                             | 88.0     |    |
| Ethyl alcohol (thinner)                                    | 1        |    |
|                                                            | 100.0    | 25 |

It is to be understood that the above examples are not to limit the scope of our invention and that various other compositions may be prepared utilizing some of the other solvents, thickeners, crystallizable water-repellent materials, and thinners or dispersing agents listed hereinabove, and various combinations of these and like materials having the necessary characteristics above described for producing the fine-grain to glass-like films characteristic of our invention.

The tests that we have found satisfactory to determine suitable solvents and thickeners (that is those capable of producing upon concentration a marked increase in viscosity sufficient to interfere with the normal crystal growth of the crystallizable water-repellent material and proper proportions thereof), are as follows: A mixture is made of the thickener and the solvent that are desired to be used, and the mixture concentrated by evaporation to the point at which the mixture shows a marked increase in viscosity such as attended by gel formation or a definite tendency to string. If the mixture either gels or strings, the solvent and thickener are suitable. The concentration of the solvent in the mixture when it reaches this point is then noted. Next, a mixture of a water-repellent crystallizable material and solvent is made and evaporated to the point at which precipitation of the crystallizable material begins. The concentration of solvent in the mixture at this point is noted.

If, at the above mentioned points of gelling or stringing and crystallizing, the concentration of the solvent in the mixture of the crystallizable material and solvent is appreciably less than the concentration of the solvent in the mixture of the thickener and solvent, the relative proportions of thickener and crystallizable material are substantially correct. If the concentrations of the solvent in the two mixtures at the point of gelling or stringing and crystallizing are close together, it may be necessary upon preparing the final waterproofing composition to decrease the concentration of the crystallizable material in order to delay its precipitation and thereby insure precipitation of the thickener before precipitation of the crystallizable material. If the mixture of thickener and solvent gels or strings at a concentration of solvent less than the concentration of solvent in the mixture of crystallizable material, the thickener will precipitate before the crystallizable material.

*Example I*

|                                                            | Per cent |             |
|------------------------------------------------------------|----------|-------------|
| Aluminum stearate (thickener)                              | 2.0      | 3.0         |
| Hydrogenated fish oil glycerides (crystallizable material) | 1.0      | 3.0         |
| Petroleum naphtha (solvent)                                | 96.5     | 93.5        |
| Cresol (thinner)                                           | 0.5      | 0.5         |
|                                                            | 100.0    | 100.0-100.0 |

*Example II*

|                                    | Per cent |  |
|------------------------------------|----------|--|
| Cumar (thickener)                  | 80.00    |  |
| Paraffin (crystallizable material) | 0.75     |  |
| Hydrogenated naphtha (solvent)     | 19.25    |  |

100.00

*Example III*

|                                                            | Grams |  |
|------------------------------------------------------------|-------|--|
| Asphalt (thickener)                                        | 20-25 |  |
| Hydrogenated fish oil glycerides (crystallizable material) | 3     |  |
| Hydrogenated fish oil acids (crystallizable material)      | 3     |  |
| Hydrogenated naphtha (solvent)                             | 100   |  |

*Example IV*

|                                  | Per cent |  |
|----------------------------------|----------|--|
| Aluminum stearate                | 1.85     |  |
| Hydrogenated fish oil glycerides | 1.00     |  |
| Carbon tetrachloride             | 96.15    |  |
| Ethyl alcohol                    | 1.00     |  |
|                                  | 100.00   |  |

*Example V*

|                                                            |       |     |
|------------------------------------------------------------|-------|-----|
| "Duco" cellulosic cement (thickener)                       | c. c. | 15  |
| Hydrogenated fish oil glycerides (crystallizable material) | gram  | 0.1 |
| Acetone (solvent)                                          | c. c. | 5   |
| Hydrogenated naphtha (solvent)                             | c. c. | 5   |

able material and solvent at the point of precipitation of the crystallizable material, the relative proportions of thickener to crystallizable material must be increased.

- 5 The above tests may be checked by microscopic examination, such as the following: A drop of the waterproofing composition containing the solvent, the water-repellent thickener, and the water-repellent crystallizable material is placed on 10 a slide and examined after solidification under a microscope with dark field illumination and a magnification of about 150 diameters. If under these conditions the film appears fine-grained to glass-like, it is a satisfactory waterproofing film, 15 indicating that the crystal growth of the crystallizable water-repellent material has been properly arrested by the thickener.

However, if definite crystals are scattered in 20 porphyritic fashion throughout the mass of the film, the proportion of crystallizable material in the mixture is too high. A new mixture with slightly smaller proportion of crystallizable material should then be tried until a satisfactory film is obtained. Alternatively, the same effect can 25 be produced in some instances, by adding to the composition a certain proportion of another miscible solvent in which the crystallizable material is more soluble and the thickener not more soluble. For example, when using the "Duco" cement 30 as the thickener with acetone as the solvent, a proportion of 0.1 gram of hydrogenated fish oil glycerides to 5 c. c. of cement gave a porphyritic structure. By adding to the mixture 1 c. c. of hydrogenated naphtha, which is a good solvent 35 for the glycerides, the film prepared with the same proportion of glycerides and cement was non-porphyritic; in other words, amorphous and glass-like.

In all of the compositions mentioned above, 40 it will be understood that the proper proportioning of the thickener and the crystallizable materials is essential. The actual amounts of thickener and crystallizable material may vary from any useful small amount up to the amounts just short of those that would normally form super-saturated solutions, that is, amounts sufficient to cause precipitation of the solids in the waterproofing composition before it is applied for use. In other words, the fine-grained to glass-like films 45 are produced by precipitation from solution, and any desired amounts of materials less than the amount that will not go into solution may be used. The actual amounts of thickener and crystallizable materials used will depend largely upon the thickness of the waterproofing film that it is 50 desired to produce and upon the degree of penetration required. The thickness of the film is proportional to the amounts of solid materials present in the composition. The penetrativeness 55 of the composition is inversely proportional to the concentration of solids therein, the greater the concentration of solids the smaller the penetrativeness of the composition and vice versa.

The waterproofing compositions of our invention 60 may be applied according to any well known methods, such as brush, spray, and immersion processes.

The waterproofing compositions of our invention 65 may be prepared by any suitable admixing of the several constituents, once the proper proportions thereof have been determined in the manner described hereinabove. For example, the thickener and the crystallizable material may be admixed in solid form and heated until at least 70 one of the materials liquefies and causes all of the

solids to mutually dissolve. The proper amount of solvent is then added to this mixture of the thickener and crystallizable material. If the thickener used is of the gel forming type, a relatively small amount, such as for example 1% or less of the thinner or dispersing agent is added to the mixture, either before or after the solvent is added, for the purpose of producing a thin penetrative mobile type of solution suitable for brushing, spraying or dipping processes.

5 Another method of preparing the composition comprises dissolving simultaneously the thickener and crystallizable material in the solvent, applying heat and agitation, if necessary, to effect solution of the solids in the solvent. Still another method of preparing the composition, when using as the thickener a gel-forming material, comprises heating the thickener and solvent mixture until a gel is formed, then adding to the gel a relatively small amount of the dispersing agent 10 to disperse the gel into a mobile colloidal solution, and then dissolving in this solution the crystallizable material.

15 From these examples it will be apparent that various other methods of preparing the compositions may be used and our invention is intended to cover any and all of such methods.

20 It is to be understood that the doctrine of equivalents applies with full force and effect to this application and the invention disclosed herein and that various modifications and changes may be made in the materials and methods used without departing from the scope of this invention. The appended claims are directed to some 25 of the novel features of the invention.

30 We claim:

1. A mobile, liquid, penetrative waterproofing composition comprising a normally solid hydrogenated fish oil, a petroleum naphtha and a natural asphalt, mixed in such proportions that 35 upon concentration of the composition said asphalt and naphtha will thicken before said hydrogenated fish oil begins to precipitate, whereby the asphalt will arrest the crystal growth of the hydrogenated fish oil when it begins to precipitate and cause the hydrogenated fish oil to precipitate in the form of extremely fine size 40 crystals.

2. A mobile, liquid, penetrative waterproofing composition that forms upon evaporation of its 45 volatile constituents a fine-grained to glass-like water-repellent film, comprising a normally solid water-repellent crystallizable organic material selected from the group consisting of fats and waxes of organic origin, an evaporating hydrocarbon solvent, and a natural asphalt, mixed in such proportions that upon concentration of the composition said natural asphalt and hydrocarbon solvent will thicken before said crystallizable material begins to precipitate, whereby said 50 natural asphalt arrests the normal crystal growth of the crystallizable material as it precipitates from said solvent, and causes said crystallizable material to precipitate in the form of extremely fine size crystals.

3. A mobile, liquid, penetrative waterproofing composition that forms upon evaporation of its volatile constituents a fine-grained to glass-like water-repellent film, comprising a normally solid water-repellent crystallizable organic material 55 selected from the group consisting of fats and waxes of organic origin, an evaporative organic solvent, and asphalt, mixed in such proportions that upon concentration of the composition said asphalt and organic solvent will thicken before 60

5

10

15

20

25

30

35

40

45

50

55

60

65

70

75

said crystallizable material begins to precipitate, whereby said asphalt arrests the normal crystal growth of the crystallizable material as it precipitates from said solvent, and causes said 5 crystallizable material to precipitate in the form of extremely fine size crystals.

4. A mobile, liquid, penetrative waterproofing composition that forms upon evaporation of its volatile constituents a fine-grained to glass-like 10 water-repellent film, comprising a normally solid water-repellent crystallizable material, an evaporative organic solvent, an an asphaltic sub-

stance, mixed in such proportions that upon concentration of the composition said asphaltic substance and organic solvent will thicken before said crystallizable material begins to precipitate, whereby said asphaltic substance arrests the 5 normal crystal growth of the crystallizable material as it precipitates from said solvent, and causes said crystallizable material to precipitate in the form of extremely fine size crystals.

10

ARTHUR F. TAGGART.  
WARLEY L. PARROTT.

CERTIFICATE OF CORRECTION.

Patent No. 2,180,971.

November 21, 1939.

ARTHUR F. TAGGART.

It is hereby certified that error appears in the printed specification of the above numbered patent requiring correction as follows: Page 4, second column, line 55, claim 2, for the word "evaporating" read evaporative; page 5, first column, line 12, claim 4, for "an an" read and an; and that the said Letters Patent should be read with this correction therein that the same may conform to the record of the case in the Patent Office.

Signed and sealed this 26th day of December, A. D. 1939.

(Seal)

Henry Van Arsdale,  
Acting Commissioner of Patents.